

106/74

May 1, 1934.

W. M. CHARMAN ET AL

1,956,895

REFRACTORY

Original Filed Feb. 27, 1932

106-69



INVENTORS  
WALTER M. CHARMAN.  
PHILIP R. WARD.

Knowles Hudson & Kent  
Atty's.

XR

## UNITED STATES PATENT OFFICE

1,956,895

## REFRACTORY

Walter M. Charman and Philip R. Ward, Cleveland Heights, Ohio; said Ward assignor to The Ferro Engineering Company, Cleveland, Ohio, a corporation of Ohio

Original application February 27, 1932, Serial No. 595,579. Divided and this application December 23, 1932, Serial No. 648,611

10 Claims. (Cl. 106-6) 69

This invention relates to improvements in refractories, particularly refractories for hot tops, and has reference especially to the chemical and physical constitution of such refractories. The 5 refractories which are the subject of the invention may be employed for the production directly of hot tops either as unitary or built up assemblies, or they may be employed as lining elements for metal casings or frames. The 10 present invention is a division of my copending application Serial No. 595,579, filed February 27, 1932.

One of the objects of the invention is the provision of a refractory of this character which 15 shall be economical to produce, and one which can be formed with a relatively high degree of accuracy in comparatively large units, the large units facilitating the assembly of the hot top or its reconditioning after use.

20 Another object is the provision of a hard rigid refractory which shall be resistant to deterioration during storage and capable of withstanding rough handling in shipment.

In the drawing:  
25 Figure 1 is a perspective view looking downwardly upon a one-piece lower lining ring for a hot top, formed in accordance with the present invention.

Fig. 2 is a transverse sectional view of the 20 same taken substantially on the line 2-2 of Fig. 1, thereby showing the ring in an inverted position.

The ring illustrated in the drawing is merely one example of a hot top refractory which 25 may be formed of the composition of the present invention. Complete hot tops consisting of refractory material alone may be built up of a plurality of molded elements, or in some cases may be molded as a unitary structure employing the present composition, and where a metal casing or frame is employed it may be protected by means of a refractory lining in one or a plurality of pieces formed of the composition of this invention. The ring herein illustrated constitutes one element of a lining for a hot top casing, being intended to be used as a substitute for a lower lining course formerly constructed of a plurality of refractory blocks, such for instance as those illustrated in Patent 40 1,804,206 to Charman et al, dated May 5, 1931.

In the drawing the ring 10 is a homogeneous, one-piece structure having a perimeter formed with a contour corresponding with the inner contour of the ingot mold with which the hot 45 top is to be used. Along its inner edge the ring

is formed with an upstanding rim 11 which is adapted to protect the inner edge of the casing ledge, by means of which the other lining elements of the hot top are supported. Any suitable means may be employed for attaching 60 the ring 10 to the casing, holes 12 being provided in the present instance for the reception of wire ties.

The ingredients which we employ in making up these refractories include a suitable aggregate that is free from any impurity that will react chemically in a harmful manner with the binder, and one in which the particles are of suitable size. The size of particles should be such that the resulting article is dense enough 65 to have considerable strength, and yet not too dense to prevent any vapors or gases, set free at the time the metal is poured, from venting off. The aggregate which we prefer to employ is silica sand of a relatively fine grade, washed 70 to remove any impurities.

While it is possible to employ various binders with different degrees of success, we have discovered after extensive experiments that by far the best results are obtained, particularly with 80 silica sand as the aggregate, from the use of sodium silicate. This is employed preferably in solution and although the moisture content may be varied more or less, we prefer to employ a silicate containing 36.47% solids and 63.53% water. 85 To produce the maximum adhesive strength of sodium silicate the ratio of sodium oxide to silicon oxide should be approximately one to three. Any material deviation from this ratio will cause a marked decrease in adhesiveness. For reasons 90 of manufacture, and to obtain the proper physical condition, we prefer to use a sodium silicate solution having a ratio of one part sodium oxide to three and twenty-five hundredths parts silicon oxide. As the alkalinity of sodium silicate increases the water resistance decreases quite rapidly. The quantity of silicate solution which should be used may be varied within workable limits, the maximum of which would be twenty 95 percent by weight.

One of the requisites of a good commercial refractory for hot tops is that it shall satisfactorily withstand hard usage, particularly in shipment, and shall remain hard and rigid after being exposed to the atmosphere for a considerable time, 105 as when stored in an unprotected or damp place. We have found that the refractories in question may be rendered practically permanent regardless of atmospheric conditions by including in the mixture from which they are molded a certain 110

74 2

1,956,896

quantity of the oxide of some metal, preferably zinc or lead. Aluminum oxide is suitable for the purpose, but on account of its greater cost, we prefer to employ instead either zinc or lead oxide.

- 5 The oxides of these metals have the effect of combining with silica and silicates to form a water resistant bond somewhat akin to a glaze except that the bond is not limited to the surface but is uniform throughout the mass of the molded article.
- 10 Although the amount of this water-proofing agent may be increased to some little extent, the proportion which we have found sufficient is one percent by weight of the whole mass. Less than five-tenths would be too little to be effective, and 15 more than five percent would increase the cost of the article without corresponding benefits.

A metal reinforcement of any suitable form is desirable but not essential. A steel rod for this purpose is indicated at 13 in Fig. 2 of the drawing.

- 20 The following proportions by weight of the ingredients named have been found in practice to produce a highly satisfactory mixture:

|                          | Approximate percentage |
|--------------------------|------------------------|
| 2. Silica sand           | 86.5                   |
| Sodium silicate solution | 12                     |
| Zinc oxide or lead oxide | 1                      |
| Water                    | .5                     |

- 25 Referring now to the method of making the refractories, the mixture is placed in the mold and compacted by ramming or otherwise. When the refractory is thus molded, it is placed in an oven and dried by baking it at a fairly high temperature. The drying should be done in an atmosphere substantially free from carbon monoxide and carbon dioxide, as for instance in an electric oven or in a muffle type oven. If a substantial amount of carbon monoxide or carbon dioxide is present the silicate is converted to a carbonate and loses the attributes of a binder, with the result that the article crumbles and has no strength.

- 30 The drying is carried far enough to expel nearly all of the moisture occurring in the mixture, both as free water and as part of the sodium silicate solution. The temperature of the drying oven should be high enough to drive off this moisture, but it should not be too high, because if a very high temperature is maintained for any considerable length of time, an excessive loss of moisture will result and the binding qualities of the silicate will be impaired to a greater or lesser extent. A temperature of 400° F. has been found to be satisfactory.

35 Immediately after the drying operation is completed the moisture content of the refractory may vary up to about one percent by weight, but preferably approximates four-tenths of one percent.

- 40 After the refractory has been stored for a considerable time some additional moisture may be taken up from the atmosphere.

- 45 If the water content of the mixture be considered to include the water in the silicate solution as well as the free water, the weight of the silicate being taken as that of the solids therein only, (hereinafter referred to as dry silicate equivalent) the ingredients of the mixture in the proportions by weight which we prefer to employ will be as follows:

|                         | Per cent |
|-------------------------|----------|
| 75 Sand                 | 86.5     |
| Dry silicate equivalent | 4.3      |
| Metal oxide             | 1        |
| Water                   | 8.1      |

After completing the drying of a refractory made from this mixture the proportion of the ingredients in their proportions by weight will be found to be substantially as follows:

|                         | Per cent |
|-------------------------|----------|
| Sand                    | 94       |
| Dry silicate equivalent | 4.7      |
| Metal oxide             | 1.1      |
| Moisture                | .4       |

In the foregoing description we have necessarily gone somewhat into detail in order to fully explain the invention, but we desire it to be understood that such detail disclosures are not to be construed as amounting to limitations, except as they may be included in the appended claims.

Having thus described our invention, we claim:

1. A refractory comprising the following ingredients uniformly distributed throughout its mass approximately the proportions by weight stated: one percent to nine percent dry sodium silicate equivalent, five-tenths percent to five percent zinc oxide and approximately eighty-five percent to ninety-eight percent an aggregate chemically inert to sodium silicate. 100

2. A refractory comprising the following ingredients in approximately the following proportions by weight: sand ninety-four percent, dry sodium silicate equivalent four and seven-tenths percent, and zinc oxide having waterproofing characteristics one percent. 105

3. A refractory comprising the following ingredients in approximately the following proportions by weight: sand ninety-four percent, dry sodium silicate equivalent four and seven-tenths percent, zinc oxide having waterproofing characteristics one percent, and moisture not over one percent. 110

4. A rigid refractory comprising the following ingredients in approximately the following proportions by weight: sand eighty-five percent to 115 ninety-eight percent, dry sodium silicate equivalent one percent to nine percent, zinc oxide five-tenths percent to five percent, and sodium carbonate between zero and minute quantities less than one percent. 120

5. A refractory comprising the following ingredients uniformly distributed throughout its mass in approximately the following proportions by weight: sand ninety-four percent, dry sodium silicate equivalent four and seven-tenths percent, and zinc oxide one percent. 125

6. A refractory comprising the following ingredients uniformly distributed throughout its mass in approximately the following proportions by weight: sand ninety-four percent, dry sodium silicate equivalent four and seven-tenths percent, zinc oxide one percent, and moisture not over one percent. 130

7. A refractory comprising the following ingredients uniformly distributed throughout its mass in approximately the following proportions by weight: sand ninety-four percent, dry sodium silicate equivalent four and seven-tenths percent, zinc oxide one percent, and moisture four-tenths of one percent. 140

8. A refractory comprising the following ingredients uniformly distributed throughout its mass in approximately the following proportions by weight: sand ninety-four percent, dry sodium silicate equivalent four and seven-tenths percent, and zinc oxide one percent, said sodium silicate being of an alkalinity approximating a ratio of one part sodium oxide to three and twenty-five hundredths parts silicate. 145

9. A refractory comprising the following ingre- 150

dients uniformly distributed throughout its mass in approximately the proportions by weight stated: one percent to nine percent dry sodium silicate equivalent, five-tenths percent to five percent zinc oxide, and approximately eighty-five percent to ninety-eight percent a silicious aggregate.

10. A refractory comprising the following ingredients uniformly distributed throughout its

mass in approximately the proportions by weight stated: one percent to nine percent dry sodium silicate equivalent, five-tenths percent to five percent zinc oxide, approximately eighty-five percent to ninety-eight percent a silicious aggregate, and 80 moisture not over one percent.

WALTER M. CHARMAN.  
PHILIP R. WARD.

10

85

15

90

20

95

25

100

30

105

35

110

40

115

45

120

50

125

55

130

60

135

65

140

70

145

75

150